# EUROPEAN PATENT SPECIFICATION

(11) **EP 2 133 438 B1**
(45) Date of publication and mention of the grant of the patent: **29.02.2012**
(21) Application number: 08017101.0
(22) Date of filing: 29.09.2008
(51) Int. Cl.: C22C 9/04

(54) **Lead-free free-cutting phosphorus brass alloy and its manufacturing method**
Bleifreie und frei schneidbare Phosphorblechlegierung und Herstellungsverfahren dafür
Alliage de laiton phosphoreux de décolletage sans plomb et son procédé de fabrication

(30) Priority: 11.06.2008 CN 200810110819; 10.09.2008 US 208117
(43) Date of publication of application: 16.12.2009
(73) Proprietor: Xiamen Lota International Co., Ltd., Jimei 361022 Xiamen (CN)
(72) Inventor: Chuankai Xu, Xiamen City Fujian Province (CN); Zhenqing Hu, Xiamen City Fujian Province (CN); Siqi Zhang, Changsha City Hunan Province (CN)
(74) Representative: Peter, Kenneth William

(56) References cited:
- GB-A- 1 437 056
- JP-A- 9 143 598
- JP-A- 57 044 491
- JP-A- 2001 064 742

## Description

### FIELD OF THE INVENTION

The present invention generally relates to a phosphorous brass alloy, especially a lead-free free-cutting phosphorous brass alloy which is applicable in forging and castings for a water supply system.

### BACKGROUND OF THE INVENTION

It is well-known that lead-containing brass alloys such as CuZn40Pb1, C36000, C3604 and C3771 usually contain 1.0-3.7wt% Pb for ensuring excellent free-cuttability.

Lead-containing brass alloys are still widely used in the manufacture of many products due to their excellent cuttability and low cost. However, Pb-contaminated steam produced by the process of smelting and casting lead-containing brass alloy, and Pb-contaminated dust produced in the process of cutting and grinding the lead-containing brass alloy, are harmful to the human body and the environment. If the lead-containing brass alloys are used in drinking-water installations such as faucets, valves and bushings, contamination of the drinking water by Pb is unavoidable. In addition, toys which are produced by Pb-containing brass alloys are more harmful, as they are touched frequently, thus increasing potential exposure to Pb.

Ingestion of lead by humans is harmful, so the use of lead is being strictly banned by law in many countries due to concerns for health and the environment. For dealing with this challenge, metallurgists and manufacturers of copper materials actively research and develop lead-free free-cutting brass alloys. Some of them use Si instead of Pb, but the cuttability is not remarkably improved and the cost increases due to the high quantity of copper. Therefore, silicon brass alloys are not commercially competitive at present. One commonly used type of lead-free free-cutting brass alloy is a bismuth brass alloy, which uses bismuth instead of Pb. Many kinds of bismuth brass alloys with high or low zinc contents have been developed, and their formal alloy grades have been registered in the United States. These kinds of brass alloys contain valuable tin, nickel and selenium, as well as bismuth. Although their cuttability is 85%-97% of lead-containing brass alloy C36000, their cost is far higher than lead-containing brass alloy C36000. Therefore, these kinds of bismuth brass alloys are not competitively priced. Bismuth brass alloys also have been researched and developed in Japan and China, and applications filed in their Patent Offices. Considering that bismuth is expensive, rare in the reserves and has poor cold and hot workability, using a bismuth brass alloy instead of a lead-containing brass alloy may be financially problematic. The invention of a free-cutting antimony brass alloy which uses Sb instead of Pb has been patented in China (ZL200410015836.5). A corresponding US (US2006/0289094) application is currently pending. Japanese Patent Application published as JP 57 044 491 discloses a phosphorus brass alloy consisting of 1~9 wt% phosphorus, 0.5~45 wt% zinc and the balance is copper. Japanese Patent Application published as JP 09143598 discloses a brass alloy composition consisting of, by weight ratio, at least 47% Cu, 15-45% Zn, 0.3 to less than 3% Al and 0.1 to 5% Si.

### DETAILED DESCRIPTION

One object of the present invention is to provide a phosphorous brass alloy which will solve the limitations of conventional brass alloys discussed above, especially the problem of lead contamination.

One object of the present invention is to provide a lead-free phosphorous brass alloy which is excellent in cuttability, castability, hot and cold workability and corrosion resistance, and which is not harmful for the environment and the human body.

One object of the present invention is to provide a lead-free free-cutting phosphorous brass alloy which is particularly applicable in forging and castings for components of water supply systems.

One object of the present invention is to provide a manufacturing method for a phosphorous brass alloy.

The objects of the present invention are achieved as follows.

The present invention is intended to provide a lead-free free-cutting phosphorous brass alloy. Considering that the solid solubility of P in the matrix of copper will be decreased rapidly with the temperature decrease, and form the brittle intermetallic compounds Cu₃P with Cu, the present invention elects P as one of the main elements for ensuring the excellent cuttability of the invented alloy and solving the limitations of conventional brass alloy discussed above, especially the environmental problem. The lead-free free-cutting phosphorous brass alloy of the present invention comprises: zinc, in amount of at least 35 wt%; copper, in an amount such that the amount of zinc and copper totals between 97.0 wt% and 99.5wt%; 0.4 to 1.6wt% P; and other elements in an amount between 0.005 and 0.6wt%, which comprise at least two other elements selected in the group consisting of Al, Si, Sb, Sn, Re, Ti and B; the balance being unavoidable impurities wherein when Pb and Fe are unavoidable impurities, the content of Pb is less than 0.02wt% and the content of Fe is less than 0.05wt%.

The present invention is intended to provide a lead-free free-cutting phosphorus brass alloy wherein the content of P is preferably ranging from 0.5 to 1.35wt%, more preferably from 0.5 to 0.9wt% and most preferably from 0.5 to 0.8wt%. The said other elements are preferably selected from Al, Si, Sb, Ti and B.

The phase compositions of the invented lead-free free-cutting phosphorus brass alloy includes primarily alpha and beta phase, and a small quantity of intermetallic compounds Cu₃P.

P is one of the main elements of the invented alloy. The beneficial effects of P include: ensuring the cuttability of the inventive alloy by the fracture of the brittle intermetallic compounds Cu₃P, which is formed by elements P and Cu; improving castability and weldability of the invented alloys as deoxidizers; and improving dezincification corrosion resistance of the invented alloy. The negative effects of P include: decreasing the plasticity of the invented alloy at room temperature; if the intermetallic compounds Cu₃P disperse in the boundary of the crystal grain, the negative influence for plasticity will be larger.

The elements Re, Ti and B in the alloy have effects on deoxidization and grain refinement. Re still can form intermetallic compounds with other elements, disperse intermetallic compounds in the interior of the crystal grain and reduce the quantity and aggregation degree of intermetallic compounds Cu₃P in the boundary of the crystal grain. The preferred content of Re, Ti and B is less than 0.02wt%.

The elements Al and Si in the alloy have the effects of deoxidization, solid solution strengthening and corrosion resistance improvement. If the content of Al and Si is higher, however, castability will decrease due to the increase in the quantity of oxidizing slag. Higher content of Si also will form brittle and hard γ-phase, which will decrease plasticity of the invented alloy. Thus, the content of Al and Si is preferably ranging from 0.1 to 0.5wt%. A small quantity of Sn is added mainly to improve dezincification corrosion resistance. Sb can also improve dezincification corrosion resistance like Sn, and furthermore is beneficial for cuttability.

The features of the inventive alloy include: (a) the phase compositions of the inventive alloy mainly include alpha phase, beta phase and intermetallic compounds, Cu₃P; (b) P is one of the main elements for ensuring the cuttability of the inventive alloy; (c) Sb is complementary for the cuttability of the inventive alloy through a small quantity of brittle intermetallic compounds, Cu-Sb; and (d) multi-component alloying and grain refinement tends to uniformly disperse the intermetallic compounds in the interior and boundary of the crystal grain, and improves plasticity of the alloy.

The cost of necessary metal materials of the invented alloy is lower than lead-free free-cutting bismuth brass alloy and antimony brass alloy, and is equivalent to lead-containing brass alloy, as a result of the selection of alloy elements, and the design of element contents.

The manufacturing process of the invented alloy is as follows: when the melt of the alloy reaches a temperature of 980 to 1000 degrees Celsius, the melt is poured into ingot moulds to form ingots for further processing.

Optionally, the raw materials used in the alloy in accordance with the invention include: electrolytic Cu, electrolytic Zn, brass scraps, Cu-P master alloy, Cu-Si master alloy, Cu-Ti master alloy, Cu-B master alloy, and optionally pure Sb, Sn, Al and Re. The raw materials are combined in a non-vacuum intermediate frequency induction electric furnace, having a quartz sand furnace lining, in the following order:

First, electrolytic Cu, brass scraps, and covering agent that enhances slag removal efficiency are added to the furnace. These materials are heated until they have melted. Then the Cu-Si master alloy, Cu-Ti master alloy, and the Cu-B master alloy are added. Thereafter, pure Sb, Sn, Al and Re are optionally added. These materials are again heated until melted, and are thereafter stirred. Then electrolytic Zn is added. The melt is stirred, and slag is skimmed from the melt. The Cu-P master alloy is then added, and the melt is stirred further. When the melt reaches a temperature of 980 to 1000 degrees Celsius, it is poured into ingot molds.

The alloy ingots may be processed in different ways according to the method of the invention. First, the ingot may be extruded at a temperature ranging from 550 to 700 degrees Celsius for about I hour with an elongation coefficient of greater than 30 to be formed, for example, into bar. Second, the ingot may be forged at a temperature ranging from 570 and 680 degrees Celsius, to be formed, for example, into a valve body, or for manufacturing other water supply system components. Third, the ingot may be remelted and cast at a temperature ranging from 980 to 1010 degrees Celsius at a pressure of 0.3 to 0.5 Mpa, for example, for manufacturing faucets.

Smelting is processed in the atmosphere when protecting with the covering agent. Casting is processed at a temperature ranging from 980 to 1000 degrees Celsius. The ingot is extruded at a temperature ranging from 550 and 700 degrees Celsius with an elongation coefficient of greater than 30, and forged at a temperature ranging from 570 to 710 degrees Celsius, or remelted to be cast at a temperature ranging from 990 and 1010 degrees Celsius by low pressure die casting.

The advantages of this manufacturing process include the following. Casting ingots (rather than extruding bars) are used directly for hot-forging, and can thus reduce manufacturing costs. Ingot remelting is favorable to control the addition of the contents when in low pressure die casting. Extruding at a greater elongation coefficient could further refine grain and intermetallic compounds such as Cu₃P and uniformly disperse intermetallic compounds and consequently decrease the negative effect on plasticity.

The inventive lead-free free-cutting phosphorus brass alloy uses P instead of Pb and has been improved on cuttability, weldability and corrosion resistance. Furthermore, by multi-component alloying, grain refinement, large deformation degree and heat-treating, the intermetallic compounds Cu₃P in granular form is dispersed in the interior and boundary of the crystal grain thereby improving workability and mechanical properties of the invented alloy. The invented alloy is applicable in spare parts, forging and castings which require cutting and particularly in forging and castings for a water supply system that requires cutting, grinding (polishing), welding and electroplating. The ingot (37mm, h 60mm) may be forged at different temperatures ranging from 570 to 700 degrees Celsius, into valves with complex structures for water supply system. The production yield by disposable mold forging is 98.6%. The results from the research of mold forging indicate the invented alloy has excellent hot workability.

### BRIEF DESCRIPTION OF THE DRAWINGS

To understand the present invention, it will now be described by way of example, with reference to the accompanying drawings in which:
FIG. 1 shows the shapes of the cutting chips formed in Examples 1, 2 and 3.
FIG. 2 shows the shapes of the cutting chips formed in Examples 4, 5, 6, 7 and 8.
FIG. 3 shows the shapes of the cutting chips formed in Examples 9 and 10.
FIG. 4 shows the shapes of the cutting chips formed in cutting lead-containing brass alloy C36000, for comparison.

### EXAMPLES

The alloy composition of examples 1 to 10 is shown in Table 1. The alloy ingots are for applications including forging, remelting and low pressure die casting, and for extruding into bar. The cuttability, castability, dezincification corrosion resistance and mechanical properties have been tested. Forging is processed at a temperature ranging from 570 to 700 degrees Celsius. The extruding is processed at a temperature ranging from 560 to 680 degrees Celsius. The low pressure die casting is processed at a temperature ranging from 980 to 1000 degrees Celsius. Stress relief annealing is processed at a temperature ranging from 350 to 450 degrees Celsius.

**Table 1 Composition of lead-free free-cutting phosphorus brass alloy (wt%)**

| Examples | Cu | P | Sb | Si | Al | Sn | Ti | B | Re | Zn |
|---|---|---|---|---|---|---|---|---|---|---|
| 1 | 60.13 | 0.42 | 0.20 | 0.24 | <0.001 | -- | -- | 0.005 | 0.003 | Balance |
| 2 | 60.11 | 0.59 | 0.10 | 0.25 | <0.001 | 0.05 | 0.02 | 0.0008 | -- | Balance |
| 3 | 57.51 | 0.69 | 0.01 | 0.04 | 0.19 | 0.04 | -- | 0.006 | -- | Balance |
| 4 | 59.18 | 0.99 | 0.01 | 0.33 | 0.05 | 0.05 | 0.01 | 0.0006 | -- | Balance |
| 5* | 59.31 | 1.00 | 0.59 | 0.28 | <0.02 | -- | -- | 0.006 | -- | Balance |
| 6* | 57.10 | 0.96 | 0.54 | 0.43 | 0.21 | -- | -- | 0.007 | -- | Balance |
| 7 | 57.94 | 0.92 | 0.01 | 0.27 | 0.16 | -- | 0.01 | 0.0008 | -- | Balance |
| 8 | 58.87 | 0.90 | 0.11 | 0.26 | 0.05 | 0.03 | -- | 0.004 | -- | Balance |
| 9 | 60.01 | 1.35 | 0.11 | 0.25 | 0.23 | -- | -- | 0.004 | 0.004 | Balance |
| 10 | 57.53 | 1.57 | 0.01 | 0.28 | 0.10 | 0.06 | 0.01 | 0.0004 | 0.002 | Balance |

| | | | | | | | | | | |
|---|---|---|---|---|---|---|---|---|---|---|
| * Not part of the inventive alloy | | | | | | | | | | |

The lead-free phosphorus brass alloy of the present invention has been tested, with results as follows:

Cuttability test:

There are several indexes and methods for testing the cuttability of the alloy. The present invention tests the cuttability by measuring the cutting resistance and comparing the shapes of cutting chips. The samples for test are in the half-hard state. The same cutting tool, cutting speed and feeding quantity (0.6mm) is approached. The relative cutting ratio is calculated by testing the cutting resistance of alloy C36000, and of the invented alloy: $\frac{Cutting resistance of alloy C ⁢ 36000}{Cutting resistance of the invented alloy} \times 100 % = relative cutting ratio$ It's assumed that the cutting ratio of alloy C36000 is 100%. FIG. 4 shows the shapes of the cutting chips formed in cutting lead-containing brass C36000 Then the cutting ratio of examples 1, 2 and 3 is ≥80% by testing the cutting resistance of alloy C36000 and examples 1, 2 and 3 of the invented alloy. FIG. 1 shows the shapes of the cutting chips formed in Examples 1, 2 and 3.The cutting ratio of examples 4, 5, 6, 7 and 8 is ≥85% by testing the cutting resistance of alloy C36000 and examples 4, 5, 6, 7 and 8 of the invented alloy. FIG. 2 shows the shapes of the cutting chips formed in Examples 4, 5, 6, 7 and 8. The cutting ratio of examples 9 and 10 is ≥90% by testing the cutting resistance of alloy C36000 and examples 9 and 10 of the invented alloy. FIG. 3 shows the shapes of the cutting chips formed in Examples 9 and 10.

Dezincification corrosion test:

Considering the invented phosphorus brass alloy will be mass produced to be castings by low pressure die casting, the samples for test are in the cast state. The samples of alloy C36000 for test are in the stress relief annealing state. The test for dezincification corrosion resistance is conducted according to PRC national standard GB 10119-88. The test results are shown in Table 2.

**Table 2 The results show dezincification corrosion resistance of lead-free free-cutting phosphorus brass alloy**

| Examples | 1 | 2 | 3 | 4 | 5* | 6* | 7 | 8 | 9 | 10 | C36000 |
|---|---|---|---|---|---|---|---|---|---|---|---|
| Dezincification layer depth/µm | 90 | 100 | 120 | 120 | 50 | 60 | 110 | 120 | 140 | 180 | 610 |

| | | | | | | | | | | | |
|---|---|---|---|---|---|---|---|---|---|---|---|
| * not part of the inventive alloy | | | | | | | | | | | |

Castability test:

Several indexes can be used to measure the castability of the alloy. The present invention uses the standard samples in volume shrinkage, cylindrical, strip and spiral for testing the castability of the lead-free free-cutting phosphorus brass alloy. For volume shrinkage samples, as may be seen in Table 3, if the face of the concentrating shrinkage cavity is smooth, and no visible shrinkage porosity in the bottom of the concentrating shrinkage cavity, it indicates castability is excellent and will be shown as "o " in Table 3. If the face of the concentrating shrinkage cavity is smooth but the height of visible shrinkage porosity in the bottom of the concentrating shrinkage cavity is less than 5mm, it indicates castability is good, and will be shown as "Δ" " in Table 3. If the face of the concentrating shrinkage cavity is not smooth and the height of visible shrinkage porosity in the bottom of the concentrating shrinkage cavity is more than 5mm, it indicates castability is poor, and will be shown as "x" in Table 3. For strip samples, the linear shrinkage rate is not more than 1.5%.For cylindrical samples, as may be seen in Table 3, if no visible shrinkage crack is shown, it indicates castability is excellent and will be shown as "o " in Table 3. If the visible shrinkage crack is shown, it indicates the castability is poor, and will be shown as "x" in Table 3. Spiral samples are for measuring the flowability of the invented alloy. The pouring temperature of each alloy is about 1000 degrees Celsius. The results are shown in Table 3. It indicates the castability of the phosphorus brass alloy is excellent.

**Table 3 The results show the castability of the lead-free free-cutting phosphorus brass alloy**

| Examples | 1 | 2 | 3 | 4 | 5* | 6* | 7 | 8 | 9 | 10 | C36000 |
|---|---|---|---|---|---|---|---|---|---|---|---|
| Volume shrinkage samples | ○ | ○ | ○ | ○ | ○ | ○ | ○ | ○ | ○ | Δ | ○ |
| Cylindrical samples | ○ | ○ | ○ | ○ | ○ | ○ | ○ | ○ | ○ | ○ | ○ |
| Melt fluid length/mm | 450 | 460 | 470 | 480 | 470 | 470 | 480 | 505 | 533 | 545 | 460 |
| Linear shrinkage rate/% | ≤1.5 | | | | | | | | | | 1.95∼2.15 |

| | | | | | | | | | | | |
|---|---|---|---|---|---|---|---|---|---|---|---|
| * not part of inventive alloy. | | | | | | | | | | | |

2. Mechanical properties test:

The samples for test are in the half-hard state. The specification is Φ6mm bar. The test results are shown in Table 4.

**Table 4 The results show the mechanical properties of the lead-free free-cutting phosphorous brass alloy**

| Examples | 1 | 2 | 3 | 4 | 5* | 6* | 7 | 8 | 9 | 10 | C36000 |
|---|---|---|---|---|---|---|---|---|---|---|---|
| Tensile strength/MPa | 503 | 510 | 505 | 520 | 540 | 530 | 515 | 520 | 510 | 500 | 485 |
| 0.2%Yeld strength/MPa | 360 | 360 | 350 | 370 | 395 | 385 | 380 | 390 | 385 | 380 | 340 |
| Elongation/% | 11.4 | 12.5 | 12.7 | 12.1 | 10.3 | 10.0 | 11.0 | 10.8 | 9.5 | 8.9 | 9 |

| | | | | | | | | | | | |
|---|---|---|---|---|---|---|---|---|---|---|---|
| * not part of inventive alloy. | | | | | | | | | | | |

3. Stress corrosion test:

The samples for test are from extruded bar, castings and forging. Stress corrosion test is conducted according to PRC's national standard GB/T10567.2-1997, Ammonia fumigation test. The test results show no crack appears in the face of the samples.

## Claims

1. A lead-free free-cutting phosphorous brass alloy comprising: zinc, in an amount of at least 35wt%; copper, in an amount such that the amount of zinc and copper totals between 97.0wt% and 99.5wt%; 0.4 to 1.6wt% P; and other elements in an amount between 0.005 and 0.6wt%, which comprise at least two other elements selected in the group consisting of Al, Si, Sb, Sn, Re, Ti and B; the balance being unavoidable impurities, wherein, when Pb and Fe are unavoidable impurities, the content of Pb is less than 0.02wt% and the content of Fe is less than 0.05wt%.

2. The lead-free free-cutting phosphorous brass alloy of claim 1, wherein the amount of P is ranging from 0.5 to 1.35wt%.

3. The lead-free free-cutting phosphorous brass alloy of claim 2, wherein the amount of P is ranging from 0.5 to 0.8wt%.

4. The lead-free free-cutting phosphorous brass alloy of claim 1, wherein the other elements are selected from the group consisting of Al, Si, Sb, Ti or B.

5. The lead-free free-cutting phosphorous brass alloy of claim 2 wherein the amount of P is ranging from 0.5 to 0.9wt%.

6. The lead-free free-cutting phosphorus brass alloy of claim 1, wherein the content of Re, Ti and B is less than 0.02 wt%.

7. The lead-free free-cutting phosphorus brass alloy of claim 1, wherein the content of Al and Si is ranging from 0.1 to 0.5wt%.

8. A manufacturing method of the lead-free free-cutting phosphorous brass alloy of any one of claims 1 to 7, wherein when the melt of said alloy reaches a temperature of 980 to 1000 degrees Celsius, the melt is poured into ingot molds to form ingots for further processing.

9. A manufacturing method of the lead-free free-cutting phosphorous brass alloy of any one of claims 1 to 7, wherein ingots are extruded at a temperature ranging from 550 to 700 degrees Celsius for about 1 hour with an elongation coefficient of greater than 30.

10. A manufacturing method of the lead-free free-cutting phosphorous brass alloy of any one of claims 1 to 7, wherein ingots are forged at a temperature ranging from 570 to 680 degrees Celsius.

11. A manufacturing method of the lead-free free-cutting phosphorous brass alloy of any one of claims 1 to 7, wherein ingots are remelted and cast at a temperature ranging from 980 to 1010 degrees Celsius at a pressure of 0.3 to 0.5 Mpa.

## Patentansprüche

1. Eine bleifreie spanbare Phosphormessinglegierung, die Folgendes beinhaltet: Zink in einer Menge von mindestens 35 Gew.-%; Kupfer in einer Menge, so dass die Menge an Zink und Kupfer zusammen zwischen 97,0 Gew.-% und 99,5 Gew.-% beträgt; 0,4 bis 1,6 Gew.-% P; und andere Elemente in einer Menge zwischen 0,005 und 0,6 Gew.-%, die mindestens zwei andere Elemente, ausgewählt aus der Gruppe, bestehend aus Al, Si, Sb, Sn, Re, Ti und B, beinhalten; wobei der Rest unvermeidbare Unreinheiten sind, wobei, wenn Pb und Fe unvermeidbare Unreinheiten sind, der Gehalt an Pb weniger als 0,02 Gew.-% beträgt und der Gehalt an Fe weniger als 0,05 Gew.-% beträgt.

2. Bleifreie spanbare Phosphormessinglegierung gemäß Anspruch 1, wobei die Menge an P im Bereich von 0,5 bis 1,35 Gew.-% liegt.

3. Bleifreie spanbare Phosphormessinglegierung gemäß Anspruch 2, wobei die Menge an P im Bereich von 0,5 bis 0,8 Gew.-% liegt.

4. Bleifreie spanbare Phosphormessinglegierung gemäß Anspruch 1, wobei die anderen Elemente aus der Gruppe, bestehend aus Al, Si, Sb, Ti oder B, ausgewählt sind.

5. Bleifreie spanbare Phosphormessinglegierung gemäß Anspruch 2, wobei die Menge an P im Bereich von 0,5 bis 0,9 Gew.-% liegt.

6. Bleifreie spanbare Phosphormessinglegierung gemäß Anspruch 1, wobei der Gehalt an Re, Ti und B weniger als 0,02 Gew.-% beträgt.

7. Bleifreie spanbare Phosphormessinglegierung gemäß Anspruch 1, wobei der Gehalt an Al und Si im Bereich von 0,1 bis 0,5 Gew.-% liegt.

8. Ein Verfahren zur Herstellung der bleifreien spanbaren Phosphormessinglegierung gemäß einem der Ansprüche 1 bis 7, wobei, wenn die Schmelze der Legierung eine Temperatur von 980 bis 1000 Grad Celsius erreicht, die Schmelze in Barrenformen eingegossen wird, um Barren zur weiteren Verarbeitung zu bilden.

9. Ein Verfahren zur Herstellung der bleifreien spanbaren Phosphormessinglegierung gemäß einem der Ansprüche 1 bis 7, wobei Barren bei einer Temperatur im Bereich von 550 bis 700 Grad Celsius für etwa 1 Stunde mit einem Ausdehnungskoeffizienten von mehr als 30 extrudiert werden.

10. Ein Verfahren zur Herstellung der bleifreien spanbaren Phosphormessinglegierung gemäß einem der Ansprüche 1 bis 7, wobei Barren bei einer Temperatur im Bereich von 570 bis 680 Grad Celsius geschmiedet werden.

11. Ein Verfahren zur Herstellung der bleifreien spanbaren Phosphormessinglegierung gemäß einem der Ansprüche 1 bis 7, wobei Barren wieder geschmolzen und gegossen werden, bei einer Temperatur im Bereich von 980 bis 1010 Grad Celsius bei einem Druck von 0,3 bis 0,5 MPa.

## Revendications

1. Un alliage de laiton phosphoreux de décolletage sans plomb comprenant : du zinc, dans une quantité d'au moins 35 % en poids ; du cuivre, dans une quantité telle que la quantité totale de zinc et de cuivre soit comprise entre 97,0 % en poids et 99,5 % en poids ; de 0,4 à 1.6 % en poids de P ; et d'autres éléments dans une quantité comprise entre 0,005 et 0,6 % en poids, comprenant au moins deux autres éléments sélectionnés dans le groupe consistant en Al, Si, Sb, Sn, Re, Ti et B ; le reste étant des impuretés inévitables, dans lequel, lorsque Pb et Fe sont des impuretés inévitables, la teneur en Pb est inférieure à 0,02 % en poids et la teneur en Fe est inférieure à 0,05 % en poids.

2. L'alliage de laiton phosphoreux de décolletage sans plomb de la revendication 1, dans lequel la quantité de P est dans la gamme allant de 0,5 à 1,35 % en poids.

3. L'alliage de laiton phosphoreux de décolletage sans plomb de la revendication 2, dans lequel la quantité de P est dans la gamme allant de 0,5 à 0,8 % en poids.

4. L'alliage de laiton phosphoreux de décolletage sans plomb de la revendication 1, dans lequel les autres éléments sont sélectionnés dans le groupe consistant en Al, Si, Sb, Re, Ti ou B.

5. L'alliage de laiton phosphoreux de décolletage sans plomb de la revendication 2 dans lequel la quantité de P est dans la gamme allant de 0,5 à 0,9 % en poids.

6. L'alliage de laiton phosphoreux de décolletage sans plomb de la revendication 1, dans lequel la teneur en Re, Ti et B est inférieure à 0,02 % en poids.

7. L'alliage de laiton phosphoreux de décolletage sans plomb de la revendication 1, dans lequel la teneur en Al et Si est dans la gamme allant de 0,1 à 0,5 % en poids.

8. Un procédé de fabrication de l'alliage de laiton phosphoreux de décolletage sans plomb d'une quelconque des revendications 1 à 7, dans lequel lorsque le bain de fusion dudit alliage atteint une température de 980 à 1 000 degrés Celsius, le bain de fusion est versé dans des lingotières pour former des lingots destinés à être traités plus avant.

9. Un procédé de fabrication de l'alliage de laiton phosphoreux de décolletage sans plomb d'une quelconque des revendications 1 à 7, dans lequel des lingots sont extrudés à une température allant de 550 à 700 degrés Celsius pendant environ 1 heure avec un coefficient d'allongement supérieur à 30.

10. Un procédé de fabrication de l'alliage de laiton phosphoreux de décolletage sans plomb d'une quelconque des revendications 1 à 7, dans lequel des lingots sont forgés à une température allant de 570 à 680 degrés Celsius.

11. Un procédé de fabrication de l'alliage de laiton phosphoreux de décolletage sans plomb d'une quelconque des revendications 1 à 7, dans lequel des lingots sont refondus et coulés à une température allant de 980 à 1 010 degrés Celsius à une pression de 0,3 à 0,5 MPa.
